

June 21, 1955

A. H. CHILDERS ET AL  
METHOD OF MAKING COMPOSITE THERMIONICALLY  
EMISSIVE CATHODE MATERIAL  
Filed Nov. 18, 1952

2,711,390



*Fig. 1*



*Fig. 2*

INVENTOR  
ALIDA H. CHILDERS  
DANIEL GOLD  
BY  
*F. Kumpf*  
ATTORNEY

1

2,711,390

**METHOD OF MAKING COMPOSITE THERMIONICALLY EMISSIVE CATHODE MATERIAL**

Alida H. Childers, New York, and Daniel Gold, Brooklyn, N. Y., assignors to Sylvania Electric Products, Inc., a corporation of Massachusetts

Application November 18, 1952, Serial No. 321,186

3 Claims. (Cl. 204—181)

This invention relates to a quick heating cathode and their method of manufacture. It particularly relates to a quick heating cathode of the type suitable for use in electron discharge devices.

The cathode assemblies of the prior art consist of a cathode sleeve usually nickel with an insulated heater centrally located inside the sleeve. The cathode becomes effective and emits electrons when the oxide coated sleeve is heated to a temperature in the neighborhood of 850° C. This is accomplished in the prior art cathode sleeves by passing current through the heater wire and bringing it up to a high temperature whereupon heat waves radiate outwardly from the heating filament and heat up the surrounding cathode sleeve. The assembly is, therefore, often called an indirectly heated cathode. Although cathodes of this type have given satisfactory service and are still doing so they have obvious disadvantages in that they are not directly heated and depend for their source of heat on the radiated heat energy emitted from a secondary source. Secondly, their efficiency is not as good as it might be as considerable energy is lost during this transmission of heat by radiation which is one of the least efficient heating methods. Thirdly, the construction is not as rugged as it might be in view of the fact that the cathode is not firmly supported and must be spaced coaxially from the heating filament and fixedly from the grid and plate if the best results are to be obtained. This is relatively difficult in view of the fact that a sudden shock or jar could disturb the relative positions of the filament and cathode sleeve as well as the sleeve and other tube elements even when these elements are properly mounted during the assembly period.

It is, therefore, an object of this invention to provide a quick heating cathode in which the heat is transferred directly to the cathode surface by conduction.

It is a further object of this invention to provide a quick heating cathode in which the power required to bring the cathode up to operating temperature will be substantially lower.

It is a further object of this invention to provide a rugged cathode construction wherein the cathode is firmly supported by the inner heating core.

It is a still further object of this invention to improve the cathode's reliability by controlling the alloy elements present in the cathode itself.

In accordance with this invention it has been found that these objects and other advantages incidental thereto can be obtained by directly coating a metal film on an insulated heater.

In the drawings which illustrate features of this invention Figure 1 is an elevation partly in section of a quick heating cathode of this invention.

Figure 2 is a schematic drawing illustrating a method of coating the insulated heater wire with a metal film in order to produce the quick heating cathode of this invention.

2

The heater of this invention is in many respects similar to an indirectly heated type heater of the prior art, that is to say, it has substantially the same number of components the most important distinction being in their relative position to one another. In this they differ only in that the metal forming the cathode sleeve itself instead of being spaced from the insulated filamentary heater is directly applied thereto. This can be seen quite clearly in Figure 1 of the drawings wherein the filamentary wire heater is shown at 10 with its insulating coating of Alundum 12 which is in turn directly coated with a nickel film 14. This is in turn coated with a normal oxide coating usually used for cathodes which is shown in the drawings at 16. In the embodiment shown this material is prepared from a triple carbonate.

With a heater of this type it is readily apparent that the cathode is necessarily quick heated in view of the fact that heat is transferred directly to the cathode surface which is in contact with the Alundum coating the filamentary wire 10. It is also readily apparent that a cathode of this type will have greater efficiency than the indirectly heated cathodes of the prior art inasmuch as the power required to bring the cathode up to operating temperature will be substantially lower. Furthermore, this cathode has a ruggedized construction in that the cathode is firmly supported by the inner core since it is attached directly thereto.

This cathode may, of course, be produced in many ways. Some steps in the production of this cathode are, of course, the same as those used in the normal construction of the prior art cathode as, for example, the heater wire 10 may be coated with the Alundum electrophoretically as is now being done in the prior art. However, once this has been accomplished it is then necessary to apply a metal film over the coating. This is more of a problem since the metal film must be continuous and since the metal must not be allowed to penetrate into the porous Alundum otherwise electrical leakage between the heater and the cathode surface will result. This would naturally lead to the production of an unsatisfactory cathode. In accordance with this invention it has been found that this metal may successfully be deposited on the porous Alundum to form a continuous metal film which does not penetrate the porous Alundum using vapor deposition techniques. One technique of this type is illustrated in Figure 2 of the drawings in which the Alundum covered heater is continuously coated with nickel from nickel carbonyl. The heater to be formed and the method to be used need not be limited to the use of nickel from nickel carbonyl. A metal film may be made from any metal which forms volatile compounds that can be decomposed below the melting point of the heater components or of the metal itself. The decomposition may be entirely thermal or aided by a reducing atmosphere such as hydrogen. For example, the metal might be a tantalum metal sheath which has been vapor deposited from tantalum pentachloride.

In accordance with the method shown in Figure 2 of the drawings a carrier gas such as helium or nitrogen is admitted to the system from tank 20, permitted to flow into supply line 22 at a constant flow rate. To this system is added nickel carbonyl in gaseous form which is obtained by vaporizing the nickel carbonyl from its liquid form which is kept in reservoir 30. This can be heated to a suitable temperature to give the desired vapor pressure by means of a heater 31. The vaporized nickel carbonyl enters the supply line 22 wherein it is transported by the carrier gas to the coating area which consists essentially of a wafer cooled condenser 32. Insulated heater wire which is present on supply spool 40

is caused to pass centrally through the condenser 32 and is positioned therein by means of pulleys 34 and 36. As the insulated wire is passing through the condenser 32 it is heated to a temperature in the neighborhood of 200° C. by means of an induction heating element as shown at 38 in the drawing. The resultant hot insulated heated wire decomposes the nickel carbonyl as it passes through the coating area. As the nickel coated wire leaves the coating area it passes over pulley 36 and into a reducing or inert atmosphere furnace 50 wherein the nickel coating is sintered. The sintered nickel coated wire then passes over pulley 52 and is spooled on reel 54.

The Alundum insulation is quite porous therefore the surface deposition conditions have to be controlled in order to maintain the proper insulation conditions between the heater and the cathode. These deposition conditions can be controlled by carrier gas flow rate and the wire temperature as it passes through the coating area. The nickel film thickness deposited can if desired be adjusted by regulating the rate of nickel carbonyl evaporation. For example, continuous nickel coating of a 0.001" tungsten wire insulated with aluminum oxide to a thickness of .003" can be successfully accomplished by using a helium flow rate of 7 cubic feet per hour and a surface temperature on the wire of approximately 200° C. By this method a nickel coating can be placed on the wire having a thickness of approximately 0.0001" to 0.0002". The resulting nickel coated wire can then be electrophoretically coated with triple carbonates to form a completed cathode assembly.

In some cases it has been found advantageous to fire the nickel coated units in hydrogen at a temperature of about 950° C. This increases the conductivity along the film and thus makes it possible to use an even thinner film of nickel.

By using these vapor deposition techniques both in the case of nickel and tantalum it has been found that no substantial diffusion of the metal will take place into the Alundum and high electrical resistance between the tungsten core and the metal film has been noted while 40 excellent conductivity along the metal film is achieved.

While the above description and drawings submitted herewith disclose a preferred and practical embodiment of the quick heating cathode of this invention it will be understood by the specific details of construction and arrangement of parts as shown and described are by way of illustration and are not to be construed as limiting the scope of the invention.

What is claimed is:

1. The method of manufacturing a composite material suitable for use as a thermionically emissive cathode in an electron discharge device which comprises electro-45 phoretically coating a heater wire with Alundum, continuously passing the cooled wire through a chamber containing nickel carbonyl while maintaining the wire in the chamber at 200° C. to obtain a nickel sheath thereon, passing the wire so treated through a chamber 10 maintained at about 950° C. cooling the treated wire and continuously coating it with a thermionically emissive material.
2. The method of manufacturing a composite material suitable for use as a thermionically emissive cathode in an electron discharge device which comprises electro-15 phoretically coating a tungsten wire with Alundum, continuously depositing nickel on said Alundum coating by passing the coated tungsten wire through a chamber containing nickel carbonyl while maintaining the wire in 20 said chamber at approximately 200° C., passing the nickel coated wire through a sintering furnace maintained at a temperature in excess of 900° C. and continuously coating the sintered material with a thermionically emissive material.
3. The method of manufacturing a composite material suitable for use as a thermionically emissive cathode in an electron discharge device which comprises electro-25 phoretically coating a tungsten wire with Alundum, continuously depositing nickel on said Alundum coating by 30 passing the coated tungsten wire through a chamber containing nickel carbonyl while maintaining the wire in said chamber at approximately 200° C., passing the nickel coated wire through a sintering furnace maintained at a temperature in excess of 900° C. and continuously 35 coating the sintered material with a triple carbonate.

References Cited in the file of this patent

UNITED STATES PATENTS

|           |            |       |               |
|-----------|------------|-------|---------------|
| 1,818,909 | Reerink    | ----- | Aug. 11, 1931 |
| 2,075,910 | Robinson   | ----- | Apr. 6, 1937  |
| 2,118,186 | Farnsworth | ----- | May 24, 1938  |
| 2,442,863 | Schneider  | ----- | June 8, 1948  |

OTHER REFERENCES

Cline et al.: Journal of the Electrochemical Society, October 1951, pp. 385 to 387.